

# UNITED STATES PATENT OFFICE.

WINFIELD S. POTTER, OF NEW YORK, N. Y.

## MAKING WROUGHT MANGANESE-STEEL CAR-WHEELS.

1,018,364.

Specification of Letters Patent. Patented Feb. 20, 1912.

No Drawing.

Application filed December 18, 1911. Serial No. 666,236.

*To all whom it may concern:*

Be it known that I, WINFIELD S. POTTER, a citizen of the United States, residing in the borough of Manhattan, city, county, and State of New York, have invented certain new and useful Improvements in Making Wrought Manganese-Steel Car-Wheels; and I do hereby declare the following to be a full, clear, and exact description of the invention, such as will enable others skilled in the art to which it appertains to make and use the same.

The purpose of my invention is to produce a manganese steel car wheel in a thoroughly wrought condition throughout and of a uniform very fine-grained and suitably hard and dense structure, particularly in the flange and tread portions of the wheel, the manufacture being so conducted as to avoid in the preliminary and in the final forming operations, various laminations and other irregularities of structure in the steel which would tend to cause irregular wearing or breakage of the wheel in service.

My improved wheel when brought to its final form and dimensions is substantially devoid of laminations and weak cleavage surfaces, and in a condition of great strength, the tread and flange portions particularly being in a state of maximum hardness consistent with the necessary toughness and shock-resistance.

In carrying out my invention, the manganese steel, while still molten, is suitably cleansed by reducing agents and by means of fluxes, and is held in the ladle prior to casting until the impurities have floated out of the metal.

The ingot is then cast of a size to produce several wheel blanks and may be of the usual tapered form. The casting is so conducted as to avoid shrinkage cavities and porosity in the main body portion of the ingot, that is to say, in that portion which is to be cut up into wheel blanks. To this end, the metal is preferably poured into molds having tops which retain the steel longer molten in the upper than in the lower portion of the mold, so that the impurities of the steel accumulate in that portion or part of the upper portion of the ingot which is to be rejected by cropping after the first stage of the forming operation. To this end, a mold having a suitable refractory top portion may be employed. Or the ingot may be produced

in accordance with my U. S. Patent No. 967,830, dated August 16, 1910.

When the ingot has been cast, as above or any other suitable manner to avoid porosity, it is permitted to freeze, and is then stripped from the mold, while still hot, and is placed in the heating furnace or soaking pit. At the time of stripping the ingot, and when it is introduced into the soaking pit, it has frozen and cooled to a temperature in the average of from about 1000° C. to about 1100° C. In the soaking pit the ingot is equalized at a temperature between about 1150° C. and 1200° C. to eliminate irregularities of composition and structure occurring during freezing and cooling. Great care is to be exercised at this juncture to avoid any coarse re-graining of the steel, and, to this end, after the ingot has been soaked within the temperature range referred to and has been equalized throughout, it is withdrawn from the soaking pit, for the reason that to retain it therein after the irregularities of composition and structure have been removed tends to bring about the coarse re-graining referred to. So also, the retaining of the ingot within the soaking pit after the irregularities of composition and structure have been removed has the further tendency to bring about, to a greater or less extent, an evolution of gases within the mass which correspondingly forces apart the crystals of the steel and thereby decreases their cohesion.

When the ingot has been brought, in the soaking pit, to the desired condition and has been removed therefrom, it is reduced to a bloom of substantially uniform cross-section throughout, and is then cut into wheel blanks of the required weight, at temperatures between 1125° C. and 1200° C., and preferably without heating it above about 1175° C. For example, the bloom may be cut by one or more rotating cutting disks into suitable wheel blanks. Instead of cutting these blanks of a length and diameter approximating the ultimate diameter of the finished wheel, I prefer, in the first instance, to roll or otherwise work the ingot when bringing it to parallel form down to a considerably lesser cross-section, so that in cutting off a blank of the requisite weight therefrom, the blank will be correspondingly longer than the ultimate average thickness of the wheel. By this expedient,

I am enabled to more accurately cut the ingot into blanks of the desired weight. The blank is then worked in its outer portions, having at this time a temperature within the range of 1125° C. to 1200° C. For example, it is placed in a suitable die, closely fitting its margin and is then subjected to heavy pressure and is thoroughly worked in its outer portions particularly, the die being of such a character as to prevent any substantial amount of stretching in this tread portion. The purpose of this preliminary working of this outer or tread portion of the blank, while at the same time preventing elongation or stretching of said tread portion is to avoid any such lamination in the finished product as would be due to internal flaws in the blank. That is to say, the thorough working of the outer or tread portion of the blank at this stage of the operation has the effect of consolidating the metal in the tread portion and eliminating any possible internal flaws or cleavage surfaces therein. The blank is then removed from the die and reheated for further forming. By a suitable rolling or pressing operation the central part or the innermost portions of the blank are suitably worked to bring them into the desired wrought condition in so far as this can be accomplished in one heating, or during one or more re-heatings, and the blank as a whole is finally brought to the desired form throughout, either in a single operation or a plurality of pressing or rolling operations.

During any of the reheating operations, the re-heating is to be so conducted as to avoid any coarse re-graining of the steel after its initial working; moreover the re-heating operations should be of but moderate duration, so that neither the temperature of the re-heating nor its duration shall have the effect of bringing about a feeble cohesion between the grains of the steel particularly in the tread and flange portions of the blank. The standard practice, therefore, as just indicated, should preferably exclude a re-heating of the tread portions of the blank at any time above 1175° C. or thereabout. If, however, the exigencies of the case require that the steel should be hotter than 1175° C., in order to suitably form the hub and web of the wheel, the entire blank may be reheated for a short time above 1175° C. (say 1200° C.).

The handling of the metal from the heat of casting through the various re-heating operations should be so conducted that after each forming operation the blank is taken quickly from the preceding operation and with as little loss of its heat as may be to a reheating furnace having the desired maximum temperature to be employed for the next forming operation. For example, the blank after having been severed from

the parallel bloom should be delivered to the next heating furnace with an average temperature of 1000° C. if possible, or with any higher temperature less than the temperature suitable for the reheating furnace at this time, which will be about 1175° C. The blank will then be brought to the desired maximum temperature for the next forming step preferably with a steadily rising temperature until the maximum temperature is reached and the piece is then only held in the furnace for a time sufficient to obtain a substantial equality of temperature throughout the blank. The same precaution should be observed with regard to each succeeding handling and reheating of the blank; as, if the blank is permitted to cool, or is placed in a furnace having a temperature much less than the intended maximum the rise of temperature in the blank to the working heat will on account of the peculiar properties of the metal be so slow as to produce a considerable crystal building and a coarse and feebly coherent re-graining of the metal.

If on account of the lack of suitable facilities the blank at any stage of its formation must be cooled to a low temperature, as for example to below a black heat before the following reheating and forming operation can be effected, the cooling and subsequent reheating should be then conducted with the following precautions:

The blank having been partially worked and having at the end of this portion of the operation a temperature of say 1050° C. or above, will be rapidly cooled (as by means of a water spray) until at a temperature of about 400° to 600° C. and may then be cooled in the air or as desired to ordinary temperatures. If the blank is worked until at a temperature ranging from say 700° to 1000° C. it may be air cooled if desired. In the subsequent reheating the blank is preferably reheated gradually to a temperature of 420° C. or thereabout; for example, it is gradually heated to between 400° to 650° C. whereupon it is charged into a furnace and the blank is then heated as rapidly as possible and preferably with a steadily rising heat to the desired temperature for the next forming operation.

The wheel is finally worked throughout at temperatures below 1075° C. and is not thereafter reheated to above 1025° C. except for very short periods of reheating.

The final working of the tread portion for the production of the greatest density and strength of metal should begin at an initial temperature throughout below 1125° C. and is preferably completed at a temperature throughout of about 900° to 1025° C. Thereafter, the tread and flange portions should not again be re-heated to a temperature above 1025° for any considerable time al-

though good results could be obtained by re-heating up to temperatures as high as 1075° C. for a very short time.

At the termination of the final working, the finished wheel may be immediately cooled, as hereinafter described, or it may be placed in a furnace having a temperature range, for example from 900 to 1075° C. but preferably about 1000° C., for a short time sufficiently to substantially equalize the temperature throughout the wheel, and the wheel is then taken from the furnace and subjected to a rapid cooling operation.

The rapid cooling operation may be carried out by immersing the entire wheel in water or in molten lead having a temperature but slightly above its melting point; or in any other suitable manner appropriate to rapidly extracting the greater part of the heat of the wheel. Or, the rapid cooling of the wheel after it has been equalized at a temperature of about 1000° C. may be executed by supporting the wheel from its central opening on a shaft by which it is rotated, and during this rotation, subjecting it to a suitable number of high pressure water jets until its temperature is reduced throughout to below 420° C.; whereupon it may be gradually or rapidly cooled to atmospheric temperature.

The machining of the running surface of the wheel and also the boring of the hub of the wheels of manganese steel may be conducted either by grinding or by bringing the parts to be machined to a temperature slightly below 420° C., say 300° C. to 420° C. and thereupon turning or boring as may be necessary. However, no portion of the mass is re-heated after the rapid cooling operation to temperatures above 420° C. or thereabout.

Having thus described my invention what I claim is:

1. The method of producing wrought manganese steel car wheels, which consists in casting a manganese ingot so as to avoid porosity, and of a size to produce several wheel blanks; permitting the ingot, after freezing, to cool to between 1000° C. and 1100° C.; reheating to between 1125° C. and 1200° C.; reducing the ingot to substantially uniform cross-section throughout its length and cutting it into blanks; immediately re-heating the blanks to not above 1200° C.; working the outer portion of the blanks and forming the hub and web portions, the final working of the hub and web portions taking place at temperatures below 1075° C. and the final working of the tread portion taking place at temperatures below 1025° C.; equalizing at between 975° C. and 1025° C.; and rapidly cooling to below 420° C.; substantially as described.

2. The method of producing wrought manganese steel car wheels, which comprises

preliminarily working a manganese steel wheel blank at temperatures between 1125° C. and 1200° C.; finally working said blank throughout at temperatures between 900° C. and 1075° C.; equalizing at about 1000° C.; 70 and rapidly cooling to below 420° C.; substantially as described.

3. The method of producing wrought manganese steel car wheels, which comprises preliminarily working a manganese 75 steel wheel blank at temperatures between 1125° C. and 1200° C.; finally working said blank throughout at temperatures between 900° C. and 1075° C.; rapidly cooling to below 420° C., and machining to form at a 80 surface temperature for the portions to be machined of between 300° C. and 420° C.; substantially as described.

4. The method of producing wrought manganese steel car wheels, which comprises reducing the ingot to substantially uniform cross-section throughout its length and cutting it into blanks at an initial temperature of about 1175° C.; thereafter working the blank into wheel form in a number 90 of forming operations with intermediate re-heating; the re-heating for each forming operation being rapidly conducted up to about 1175° C., and for a period of moderate duration; finishing the working at temperatures below 1075° C.; and finally cooling rapidly to below 420° C.; substantially as described.

5. The method of producing wrought manganese steel car wheels, which comprises reducing the ingot to substantially uniform cross-section throughout its length and cutting it into blanks at an initial temperature of about 1175° C.; thereafter working the blank into wheel forms in a number 100 of forming operations with intermediate re-heating; the re-heating for each forming operation being rapidly conducted up to about 1175° C., and for a period of moderate duration; and the temperature from one 110 forming operation to the next re-heating not being permitted to drop below an average of about 1000° C.; finishing the working at temperatures below 1075° C.; and finally cooling rapidly to below 420° C.; substantially 115 as described.

6. The method of producing wrought manganese steel car wheels, which comprises preliminarily working a manganese steel wheel blank at temperatures between 1125° and 1200° C.; completing the working of all parts of the blank thereafter at temperatures below 1075° C.; and finally cooling rapidly to below 420° C.; substantially 120 as described.

7. The method of producing wrought manganese steel car wheels, which comprises primarily working a manganese steel wheel blank at temperatures between 1125° C. and 1200° C.; completing the working of 130

all parts of the blank thereafter at temperatures below 1075° C.; equalizing at between 900° C. and 1075° C.; and finally cooling rapidly; substantially as described.

- 5 8. The method of producing wrought manganese steel car wheels, which comprises preliminarily working a manganese steel wheel blank at temperatures between 1125° C. and 1200° C.; completing the working of all parts of the blank thereafter at temperatures below 1075° C.; and, finally cooling rapidly from about 1000° C. to below 420° C.; substantially as described.
- 10 9. The method of producing wrought manganese steel car wheels, which com-

prises consolidating the outer portions of a manganese steel wheel blank by compressing at between 1125° C. and 1200° C.; working the blank to wheel form; then working the blank throughout at temperatures below 20 1075° C.; and cooling rapidly from about 1000° C. to below 420° C.; substantially as described.

In testimony whereof I affix my signature, in presence of two witnesses.

WINFIELD S. POTTER.

Witnesses:

M. A. BILL,  
JOHN C. PENNIE.